

## UNITED STATES PATENT OFFICE

2,385,137

PREPARATION OF DIAMOND DIES FOR  
WIRE DRAWING

Alan Edgar Jones, Prescot, England, assignor to  
British Insulated Cables Limited, Prescot, Eng-  
land, a British company

No Drawing. Application April 21, 1945, Serial  
No. 589,704. In Great Britain May 18, 1944

2 Claims. (Cl. 51—293)

The preparation of diamond dies for use in wire drawing includes the steps of drilling the hole, shaping the drilled hole and finishing it to the exact size required. Each of these steps is performed by producing relative rotation between the diamond and a needle or wire, generally accompanied by a slow or intermittent endwise reciprocation. Diamond powder is utilised as the cutting agent, working between the needle or wire and the diamond. The powder is applied by using a liquid or semi-liquid material as a carrier.

For the drilling operation a steel needle is used with one end working in the hole formed in the diamond. A mixture of fine diamond powder with a carrier, for instance olive oil or lanoline, is fed from a small scoop or palette on to the needle in the hole. For the other operations the needle or wire passes through the hole and may be parallel with the axis of the hole or inclined thereto. When a wire is used it is held at both ends. The feeding of the diamond powder is carried out in substantially the same manner in each case. Each process is a slow one, for instance in drilling stones of a certain weight and size of die hole the rate of piercing may be of the order of 1 mil per hour.

By the present invention the process is improved by using as a carrier the liquid cyclohexanol. In this improved process the speed of removal of material in the hole is greatly increased. For instance, in drilling operations in comparable conditions the average rate of piercing when using olive oil or lanoline as the carrier was 1 mil per hour, whereas when using cyclohexanol the rate increased to 8 mils per hour. In the shaping operation the rate of increase of diameter of the die channel was increased from 0.25 mil per hour for olive oil or lanoline to 3.0 mils per hour for cyclohexanol. In addition to these improvements a smoother surface and a better shape in the hole is obtained, so that less work has to be done in the final operations. It will be understood that from time to time it is necessary to restore the shape of the point of the needle: this is required to be done less frequently when using cyclohexanol. When using olive oil as the carrier in certain conditions when drilling, stoppage for regrinding is necessary at intervals as short as 10 minutes. In the same conditions when using cyclohexanol the interval time is increased to 30 or 40 minutes in the early stages of a drilling and up to 60 minutes in the later stages.

There is the further advantage that with cyclo-

hexanol it is much easier than with the other carriers mentioned to clean the surface of the diamond, or of the wire or the needle when this is required to be done.

5 The action of the carrier is not fully understood, but it is suggested that when using olive oil or lanoline as a carrier there is a lubricating condition in addition to the carrying action due to the presence of a cushion between the diamond particles and the wall of the hole which retards the rate of cutting; whereas when using cyclohexanol the desired carrying action is obtained without lubrication as compared with the other materials mentioned and the absence of the cushion permits the sharp cutting edges of the diamond powder particles to have free access to the wall of the hole. It is further suggested that in drilling there is movement of the diamond particles within the body of the carrier liquid 10 away from the base of the hole where the needle operates, and that advantageous action is obtained by the rapid and regular replacement of these particles by others suspended in the carrier, and that this occurs more effectively when 15 the carrier is cyclohexanol, than with the previously known carrier materials. Again, where the movement of the cutting particles away from the base of the hole is rendered slow by the retarding effect of viscosity in the carrier, as with 20 liquids such as olive oil, a condition is created in which the broken down particles of diamonds cause a burnishing rather than a cutting action 25 to take place on the surfaces of the hole, resulting in the production of a flat polished base to 30 the hole which is resistive of further penetration. 35 This provides a possible explanation of the reduction in frequency of regrinding necessary when using cyclohexanol, since the increased resistance to penetration is productive of an increased rate of wear of the needle point.

40 The cyclohexanol is mixed with the diamond powder and the mixture applied to the wire or the needle. It is found that small additional quantities of cyclohexanol must generally be added 45 from time to time to make up for the occurrence of a small loss of the liquid. This is done by feeding with a small brush on to the wire or the needle in the hole. This loss may be due in part to evaporation (although this is small in 50 any case), or it may be due to the throwing out of the liquid from the hole by centrifugal force or to the need for thinning down the mixture. Good proportions for the mixture are about five parts of cyclohexanol to one part of diamond powder by volume. The ratio may be varied to

some small extent depending upon the work being done. For instance, in the early stage of drilling, when a large surface area of needle point is in use, the dispersion may be more concentrated i. e. may contain a larger proportion of diamond powder; in the later stage when there is a reduced surface area of needle point in use the dispersion may be less concentrated.

If a substantial part of the relative rotation is obtained by the movement of the die an enclosing cap is necessary or advisable to prevent excessive loss of liquid from the hole. A machine working with the axis of rotation vertical, or approximately vertical, gives superior results as compared with a machine in which the axis of rotation is horizontal.

For the final operations it may be advanta-

geous to resort to the use of olive oil or lanoline as a carrier to obtain the smaller rate of removal of material as the final dimensions are being arrived at.

6. What I claim as my invention is:

1. In the process of preparing a hole in a diamond die for wire drawing, using as the operating member a needle or wire moved relative to the diamond, the step of feeding the space between the operating member and the surface of the hole with diamond powder suspended in cyclohexanol.

2. A cutting agent for use in preparing holes in diamond dies consisting of a suspension of diamond powder in cyclohexanol.

ALAN EDGAR JONES.